# EUROPEAN PATENT SPECIFICATION

(11) **EP 2 650 886 B1**
(45) Date of publication and mention of the grant of the patent: **05.05.2021**
(21) Application number: 11832051.4
(22) Date of filing: 14.10.2011
(51) Int. Cl.: H01F 1/057, H01F 7/02, B22F 3/16, H01F 41/02

(54) **PREPARATION METHOD FOR HIGH-CORROSION RESISTANT SINTERED NDFEB MAGNET**
HERSTELLUNGSVERFAHREN EINES NDFEB-SINTERMAGNETEN VON HOHER KORROSIONSBESTÄNDIGKEIT
PROCÉDÉ DE PRÉPARATION D'UN AIMANT NDFEB FRITTÉ PRÉSENTANT UNE RÉSISTANCE ÉLEVÉE À LA CORROSION

(30) Priority: 15.10.2010 CN 201010515292
(43) Date of publication of application: 16.10.2013
(73) Proprietor: Ningbo Institute Of Material Technology And Engineering Chinese Academy of Sciences, Ningbo, Zhejiang 315201 (CN); Robert Bosch GmbH, 70442 Stuttgart (DE)
(72) Inventor: CHEN, Renjie, Zhejiang 315201 (CN); YAN, Aru, Zhejiang 315201 (CN); LI, Dong, Zhejiang 315201 (CN); ZHOU, Qiaoying, Zhejiang 315201 (CN); ZHOU, Longjie, Shanghai 200335 (CN); WILDE, Alexandra, 70839 Gerlingen-Schillerhöhe (DE)
(74) Representative: Bee, Joachim
(86) International application number: PCT/CN2011/080771
(87) International publication number: WO 2012/048654

(56) References cited:
- WO-A1-2010/063143
- CN-A- 101 266 857
- CN-A- 101 320 609
- CN-A- 101 320 609
- CN-A- 101 499 346
- CN-A- 101 499 346
- CN-A- 101 615 461
- CN-C- 100 480 412
- JP-A- 2006 210 893

## Description

### TECHNICAL FIELD

The present invention relates to a preparation process of high corrosion resistant sintered NdFeB magnets.

### BACKGROUND ART

In 1983, Sagawa et al in Sumitomo Special Metals Corporation of Japan firstly employed a powder metallurgy process to develop a high-performance NdFeB permanent magnetic material, which proclaims the birth of the third generation of rare earth permanent magnetic material. Compared with the previous rare earth permanent magnetic material, NdFeB-based rare earth permanent magnetic material has the following advantages: firstly, iron is used as a main component which is cheap in price, and Nd which has a smaller content in the magnet is also a widely available rare earth metal, thus the price of the permanent magnets is remarkably reduced; secondly, iron atoms rich in high magnetic moment render the saturation magnetic polarization of the material reaches 4πMs = 1.6T, magnetic crystal anisotropy field µ₀Hₐ = 7T, thus a record high maximum magnetic energy product is achieved, the theoretical value of the maximum magnetic energy product is as high as 512 kJ/m³ (64MGOe); in addition, Nd₂Fe₁₄B has a tetragonal structure which tends to form a phase. The practically used sintered Nd-Fe-B magnets are mainly composed of a main phase of hard magnetic phase Nd₂Fe₁₄B, a secondary phase of boron-rich phase and Nd-rich phase etc.

As the permanent magnetic material with excellent overall performances as known hitherto, NdFeB permanent magnetic material has been a research focus of worldwide researchers since its invention, and has been used in various aspects of life. In the 21st century, with the rapid development of high-tech industries such as computers, electronics and information technologies, production of NdFeB magnets enters a period of rapid growth.

Replacing ferrite magnets with sintered NdFeB magnets has become an important development trend of electric motor industry, especially for electric motors used in electric vehicles and hybrid power vehicles.

With the expansion of the application field of NdFeB magnets, its working environment is becoming more and more complex, requirements on the material's corrosion resistance are higher. Especially, when used in the generators and electric motors, magnets are often required to have a good corrosion resistance at high temperatures.

Common NdFeB magnets have a low corrosion resistance against air (mainly O₂), moisture and salt. This disadvantage has seriously hampered its application in generators and electric motors.

Therefore, it is indeed necessary to provide new NdFeB magnets having a good corrosion resistance, so as to overcome the disadvantages in prior art.

JP 2006 210893 A describes a rare earth permanent magnet material based on an R-Fe-Co-B-Al-Cu system wherein R is at least one element selected from Nd, Pr, Dy, Tb, and Ho, 15 to 33% by weight of Nd being contained. At least two compounds selected from M-B, M-B-Cu and M-C compounds (wherein M is Ti, Zr or Hf) and an R oxide have precipitated within the alloy structure as grains having an average grain size of up to 5 µm which are uniformly distributed in the alloy structure at intervals of up to 50 µm.

CN 101 320 609 A describes a high corrosion resistant sintered NdFeB magnet with a grain boundary reconstruction, characterized in that the magnet composition is: NdₑFe_{100-e-f-g}B_{f}M_{g}, wherein 6≤e≤24, 5.6≤f≤7, 0.03≤g≤8, M is Dy, Tb, Pr, Sm, Yb, La, Co, Ni, Cr, Nb, Ta, Zr, Si, Ti, Mo, W, V, Ca, Mg, Cu, Al, Zn, Ga, Bi, Sn, In elements in one or several.

CN 100 480 412 C discloses a single-texture magnetic RE-Fe-B compound consisting of Nd 13-27 wt%, light RE 7-20 wt%, heavy RE 5-13.5 wt%, Fe 57-65 wt%, B 1-1.2 wt%, Co 3-11 wt%, except inevitable impurity, wherein the light RE is a composition of Ce and Pr and includes at least Ce 0-11.5 wt% or Pr 0-15 wt%, and the heavy RE is a composition of Dy and Tb and includes at least Dy 0-11.5 wt% or Tb 0-8 wt%, and the light RE accounts for 0-60 wt% of the total content of light RE and heavy RE.

### SUMMARY OF THE INVENTION

In order to overcome the defects of existing NdFeB magnets, the present invention provides high corrosion resistant sintered NdFeB magnets.

Described is a high corrosion resistant NdFeB sintered magnet, wherein the composition of the magnet by mass% is NdₓRₓ₁Fe_{100-(x + x1 + y + y1 + z)}T_{y}M_{y1}B_{z}, wherein 24 ≤ x ≤ 33, 0 ≤ x1 ≤ 15, 1.43 ≤ y ≤ 16.43, 0.1 ≤ y1 ≤ 0.6, 0.91 ≤ z ≤ 1.07, R is one or more selected from the group consisting of Dy, Tb, Pr, Ce and Gd, T is one or more selected from the group consisting of Co, Cu and Al, M is one or more selected from the refractory metal group consisting of Nb, Zr, Ti, Cr and Mo, and M is mainly distributed within the grain boundary phase of the NdFeB magnet. The present invention provides a preparation process of the NdFeB magnet, according to claim 1, said process comprising:
providing a main phase alloy powder, the composition of the main phase alloy by mass% is NdₓRₓ₁Fe_{100-(x + x1 + y + z)}T_{y}B_{z}, wherein 24 ≤ x ≤ 33, 0 ≤ x1 ≤ 15, 1.43 ≤ y ≤ 16.43 , 0.91 ≤ z ≤ 1.07, R is one or more selected from the group consisting of Dy, Tb, Pr, Ce and Gd, T is one or more selected from the group consisting of Co, Cu, and Al;
providing an auxiliary phase alloy powder, the composition of the auxiliary phase alloy by mass% is NdₓRₓ₁Fe_{100-(x + x1 + y + y1 + z)}T_{y}M_{y1}B_{z}, wherein 24 ≤ x ≤ 63, 0 ≤ x1 ≤ 19, 1.43 ≤ y ≤ 16.43, 6 ≤ y1 ≤ 18, 0.91 ≤ z ≤ 1.07, R is one or more selected from the group consisting of Dy, Tb, Pr, Ce and Gd, T is one or more selected from the group consisting of Co, Cu, and Al, and M is one or more selected from the refractory metal group consisting of Nb, Zr, Ti, Cr and Mo;
mixing the main phase alloy powder with the auxiliary phase alloy powder, wherein the content of the auxiliary phase alloy powder is 1 - 10% by the total mass;
press-molding the mixed powder in a magnetic field into a preform, and then
isostatic pressing was performed at a pressure above 200MPa;
placing the molded preform in a high-vacuum sintering furnace for sintering, so as to obtain sintered magnet, wherein the refractory metal group is mainly distributed within the grain boundary phase of the NdFeB magnet.

Compared with the preparation process of NdFeB magnets in the prior art, in the present preparation process of NdFeB magnets, adding only a small amount even trace amount of refractory metals into the sintered NdFeB magnets significantly improves the high-temperature corrosion resistance of the NdFeB magnets. At the same time, the addition of refractory metals would not impair the magnetic properties of NdFeB magnets.

### DESCRIPTION OF THE PREFERRED EMBODIMENTS

In order to improve the high temperature corrosion resistance of the sintered NdFeB magnets, two technical routes can be taken. One is to improve the intrinsic corrosion resistance of the NdFeB magnets, and the other is to apply a coating on the surface of the magnets. However, the durability of the corrosion resistant coating is usually insufficient to meet the requirements of practical use.

The present invention employs the first technical route, that is, to improve the intrinsic corrosion resistance of the NdFeB magnets.

In the present invention, by adding refractory metals into the sintered NdFeB magnets using a bi-phase alloy sintering method, the refractory metals are added to the grain boundary phase of the NdFeB magnets, so as to improve the high temperature corrosion resistance of the NdFeB magnets. The added refractory metals may be Nb, Zr, Ti, Cr or Mo, preferably Nb, Zr or Ti. The chemical composition of the finally obtained sintered NdFeB magnets of the present invention can be readily determined by existing analytical methods.

Compared with Nd, Ce is more abundant in the earth crust and has a lower cost, therefore Ce is often used in the NdFeB magnets to replace Nd, so as to reduce the cost of the product.

Gd is a kind of heavy rare earth element, and is useful for stabilizing the magnetic properties of the magnets material at high temperatures.

The bi-phase alloy sintering method is a recently developed new method for producing sintered NdFeB magnets material. The method uses an alloy of two components, after coarsely crushing the alloy to a certain degree, the two components are mixed by a certain ratio, oriented, press molded, and then magnets are produced through sintering, tempering, and detection.

In the present invention, by means of the bi-phase alloy sintering method, adding only a small amount even trace amount of refractory metals into the sintered NdFeB magnets significantly improves the high-temperature corrosion resistance of the NdFeB magnets.

This is because in the bi-phase alloy sintering method, the main-phase alloy does not melt substantially, and the refractory metals contained in the auxiliary phase alloy are mainly distributed in the grain boundary phase in the magnets. In this way, only a small amount of refractory metals can significantly improve the high-temperature corrosion resistance of the magnets. Meanwhile, since the refractory metals are mainly distributed in the grain boundary phase, the magnetic properties of NdFeB magnets would not be impaired.

Thus, under the condition that the magnetic properties are substantially not affected, the addition of only a small amount of refractory metals can significantly improve the high-temperature corrosion resistance of the NdFeB magnets

Although there are attempts to add refractory metals into the NdFeB magnets in the prior art, these attempts often add refractory metals into the main phase alloy. As a result, a large amount of refractory metals are used, but the improvement of high-temperature corrosion resistance is not obvious, and the magnetic properties of the magnets are adversely harmed.

The inventive concept of modification by the grain boundary phase proposed in the present invention is based on the experience in the production of the sintered NdFeB magnets material, since in the grain boundary phase alloy (auxiliary phase alloy) designed by the present invention, the content of rare earth is high, its melting point is lower than the that of the main phase in the sintered magnets. At sintering temperature, the grain boundary phase is a liquid phase, and the main phase is still a solid phase, thus the elements in the grain boundary phase alloy hardly penetrate into the main phase. This is decided by the characteristics of NdFeB sintering and the bi-phase alloy sintering process.

As an exemplary embodiment of the production of NdFeB magnets of the present invention by means of bi-phase alloy sintering method, NdFeB magnets of the present invention can be produced by the following steps:
- providing a main phase alloy, the main phase alloy is formed into a NdFeB ingot alloy by means of a casting process or formed into a NdFeB strip by means of a strip casting process, the main phase alloy is crushed using a hydrogen decrepitation method or a mechanical crushing method, then milled into powders by a jet mill or a ball mill, thus main phase alloy powders having an average particle diameter of 2 - 5µm are obtained;
- providing an auxiliary phase alloy powder, the auxiliary phase alloy is formed into an ingot alloy by means of arc melting or formed into a strip by means of a strip casting process or formed into a quick quenching band by means of a quick quenching process, the auxiliary phase alloy is crushed using a hydrogen decrepitation method or a mechanical crushing method, then milled into powders by a jet mill or a ball mill, thus auxiliary phase alloy powders having an average particle diameter of 2 - 5µm are obtained;
- mixing the main phase alloy powder with the auxiliary phase alloy powder, wherein the content of the auxiliary phase alloy powder is 1 - 10% by the total mass, then the powders are mixed homogeneously;
- press-molding the mixed powder in a magnetic field into a preform, then isostatic pressing was performed at a pressure above 200MPa;
- placing the molded preform in a high-vacuum sintering furnace for sintering at a temperature between 1040-1120°C for 2-5 hours, so as to obtain sintered magnets.

During the above isostatic pressing treatment, the higher the pressure is, the more beneficial it would be for the properties of the material, but an overhigh pressure would impose more requirements on the safety facilities, and also result in a volume increase of the apparatus, resulting in increased production costs.

As for the sintering treatment, for example, in the NdFeB magnets preparation process of the present invention, the sintering in the high vacuum sintering furnace can be carried out in the following manner: sintering at 1040-1120°C for 2-5 hours to obtain sintered magnets.

Depending on the specific conditions, the magnets may be primarily tempered at 850-950°C for 2-3 hours, then secondarily tempered at 450-550°C for 2-5 hours, so as to obtain sintered magnets.

The tempering treatment is optional. Primary tempering and secondary tempering can be carried out either one of them or both, or neither of them.

The present invention is now described in detail with reference to the following examples: However, the examples are only for illustrative purposes and do not limit the present invention in any manner.

### Example 1

The main phase alloy with a composition of Pr₆Nd₂₄Fe_{67.45}Dy_{0.5}Co_{0.6}Cu_{0.04}Al_{0.25}Zr_{0.2}B_{0.96} (mass percent) was formed into strips by means of the strip casting process, and then formed into powders having an average particle diameter of 3.6 microns using the hydrogen decrepitation and jet milling process. The powders were oriented in a magnetic field of 2T and press molded. Under a pressure of 300MPa, isostatic pressing was performed for 20 seconds. The preform was then placed in a vacuum furnace at 1080°C and sintered for 2 hours, followed by two stage heat treatments, wherein the primary heat treatment was performed at 875°C for 2 hours; and the secondary heat treatment was performed at 560°C for 2 hours. Thus, master alloy sintered magnets were obtained. The magnetic characteristics of the produced master alloy magnets are summarized in Table 1.

The auxiliary phase alloy with a composition of Pr₆Nd₂₄Fe_{47.45}Dy_{0.5}Nb₂₀Co_{0.6}Cu_{0.04}Al_{0.25}Zr_{0.2}B_{0.96} (mass percent) was formed into strips by means of the strip casting process, and then formed into powders having an average particle diameter of 3.6 microns using the hydrogen decrepitation and jet milling process. The auxiliary alloy powder which accounts for 1 mass% of the total mass were added into the above main phase alloy powders and mixed homogeneously, the composition of the final alloy is: Pr₆Nd₂₄Fe_{67.25}Dy_{0.5}Nb_{0.2}Co_{0.6}Cu_{0.04}Al_{0.25}Zr_{0.2}B_{0.96} (mass percent). Subsequently, the same orientation, pressure molding process, isostatic pressing, vacuum sintering, and heat treatment as applied to the master alloy was applied to obtain the final magnets. The magnetic characteristics (20°C) of the final magnets containing the auxiliary phase alloy are summarized in Table 1.

The master alloy magnets and the final magnets containing the auxiliary phase alloy were respectively formed into magnets of two specifications: Φ10mm × 10mm and Φ15mm × 3mm, five pieces of each specification, 20 in total. Subsequently, HAST tests were carried out at the following experimental conditions: 130°C, 0.26MPa, 168 hours. The mass loss of the master alloy magnets and the final magnets containing the auxiliary phase alloy are summarized in Table 1.

Corrosion resistance tests:
Autoclave tests were performed at 130°C and a relative humidity of 95% for 168 hours, and high-temperature corrosion resistance of the produced magnets was evaluated.

The test results are shown in Table 1, and the data indicates that the surface corrosion of NdFeB magnets produced in Example 1 is significantly improved. Specifically, in the autoclave test, at 130°C and a relative humidity of 95%, for 168 hours, the average mass loss decreased from 1.71 mg/cm² to 0.19 mg/cm².

Under the same test conditions, the surface corrosion of typical commercially available sintered NdFeB magnets is usually as high as 2 mg/cm².

Magnetic flux loss after aging at a high temperature:
After aging at 150°C for 1000 hours, the magnetic flux loss of the magnets was measured.

Under the same aging conditions, the magnetic flux loss of the sintered NdFeB magnets of the present invention was only 0.77%.

Typically, the requirement on the magnetic flux loss of the commercially available magnets is that the magnetic flux loss within 3 hours at the working temperature is less than 5%. It can be seen that the performance of the magnetic flux loss of the magnets of the present invention is far superior to this requirement.

**Table 1 Comparison of the magnetic properties and the average mass loss between the master alloy magnets and the final sintered magnets containing 1 mass% of the auxiliary alloy**

| | Remanence | Coercivity | Magnetic energy product | Average mass loss (mg/cm²) |
|---|---|---|---|---|
| Master alloy magnets | 1.35 T (13.5 kGs) | 939 kA/m (11.8 kOe) | 351.7 kJ/m³ (44.2 MGOe) | 1.71 |
| Final magnets | 1.345 T (13.45 kGs) | 927.1 kA/m (11.65 kOe) | 347 kJ/m³ (43.6 MGOe) | 0.19 |

### Example 2

The main phase alloy with a composition of Nd₂₄Fe_{67.48}Tb_{0.8}Dy₅Co_{1.0}Zr_{0.2}Cu_{0.23}Al_{0.3}B_{0.99} (mass percent), and an auxiliary phase alloy with a composition of Nd₄₀Fe_{31.48}Tb_{0.8}Dy₅Co_{1.0}Zr_{0.2}Nb₂₀Cu_{0.23}Al_{0.3}B_{0.99} (mass percent) were formed into strips respectively by means of the strip casting process, and then formed into powders having an average particle diameter of 3.5 microns using the hydrogen decrepitation and jet milling process. The auxiliary alloy powder which accounts for 1 mass% of the total mass were added into the above main phase alloy powders and mixed homogeneously, the composition of the finally obtained alloy is: Nd_{24.16}Fe_{67.12}Tb_{0.8}Dy₅Co_{1.0}Nb_{0.2}Zr_{0.2}Cu_{0.23}Al_{0.3}B_{0.99} (mass percent). Subsequently, the master alloy powders and the final alloy powders were molded and oriented in a magnetic field of 2T and a 300MPa isostatic pressing was performed for 20 seconds. The produced preforms were then respectively placed in a vacuum furnace at 1090°C and sintered for 2 hours, followed by two stage heat treatments, wherein the primary heat treatment was performed at 900°C for 2 hours; and the secondary heat treatment was performed at 500°C for 2 hours. Thus, master alloy sintered magnets and final sintered magnets were obtained. The magnetic characteristics (20°C) of the produced master alloy magnets and the final sintered magnets are summarized in Table 2.

The master alloy magnets and the final magnets containing the auxiliary phase alloy were respectively formed into magnets of two specifications: Φ10mm × 10mm and Φ15mm × 3mm, five pieces of each specification, 20 in total. Subsequently, HAST tests were carried out at the following experimental conditions: 130°C, 0.26MPa, 168 hours. The mass loss of the master alloy magnets and the final magnets containing the auxiliary phase alloy are summarized in Table 2.

Corrosion resistance tests:
Autoclave tests were performed at 130°C and a relative humidity of 95% for 168 hours, and high-temperature corrosion resistance of the produced magnets was evaluated.

Test results are shown in Table 2, and the data indicates that the surface corrosion of NdFeB magnets produced in Example 2 is significantly improved. Specifically, in the autoclave test, at 130°C and a relative humidity of 95%, for 168 hours, the average mass loss decreased from 1.6 mg/cm² to 0.13 mg/cm².

**Table 2 Comparison of the magnetic properties and the average mass loss between the master alloy magnets and the final sintered magnets containing 1 mass% of the auxiliary alloy**

| | Remanence | Coercivity | Magnetic energy product | Average mass loss (mg/cm²) |
|---|---|---|---|---|
| Master alloy magnets | 1.19 T (11.9 kGs) | 2005 kA/m (25.2kOe) | 279.3 kJ/m³ (35.1 MGOe) | 1.6 |
| Final magnets | 1.18 T (11.8 kGs) | 1950 kA/m (24.5 kOe) | 274.5 kJ/m³ (34.5 MGOe) | 0.13 |

It can be seen from the above examples that, in the present invention, by adding a small amount of refractory metals in a unique way, the high temperature stability and corrosion resistance of the magnets are significantly improved, and the magnetic properties of the magnets only slightly decreased.

This technical effect is never achieved in the prior art, and it can not be easily inferred by those skilled in the art.

## Claims

1. A preparation process of high corrosion resistant sintered NdFeB magnet, said process comprising:
providing a main phase alloy powder, the composition of the main phase alloy by mass% is NdₓRₓ₁Fe_{100-(x+x1+y+z)}T_{y}B_{z}, wherein 24 ≤ x ≤ 33, 0 ≤ x1 ≤ 15, 1.43 ≤ y ≤ 16.43 , 0.91 ≤ z ≤ 1.07, R is one or more selected from the group consisting of Dy, Tb, Pr, Ce and Gd, T is one or more selected from the group consisting of Co, Cu, and Al;
providing an auxiliary phase alloy powder;
mixing the main phase alloy powder with the auxiliary phase alloy powder, wherein the content of the auxiliary phase alloy powder is 1 - 10% by the total mass;
press-molding the mixed powder in a magnetic field into a preform, then isostatic pressing was performed at a pressure above 200MPa;
placing the molded preform in a high-vacuum sintering furnace for sintering, so as to obtain sintered magnet, wherein the refractory metal group is mainly distributed within the grain boundary phase of the NdFeB magnet, **characterised in that** the composition of the auxiliary phase alloy by mass% is NdₓRₓ₁Fe_{100-(x + x1 + y + y1 + z)}T_{y}M_{y1}B_{z}, wherein 24 ≤ x ≤ 63, 0 ≤ x1 ≤ 19, 1.43 ≤ y ≤ 16.43, 6 ≤ y1 ≤ 18, 0.91 ≤ z ≤ 1.07, the content of Fe is 100 - (x + x1 + y + y1 + z), and R is one or more selected from the group consisting of Dy, Tb, Pr, Ce and Gd, T is one or more selected from the group consisting of Co, Cu, and Al, M is one or more selected from the refractory metal group consisting of Nb, Zr, Ti, Cr and Mo.

2. The preparation process of claim 1, wherein the average particle diameter of the main phase alloy powder is 2-5 µm.

3. The preparation process of claim 1, wherein the average particle diameter of the auxiliary phase alloy powder is 2-5 µm.

4. The preparation process of claim 1, wherein the molded preform is sintered at 1040-1120 °C for 2-5 hours in a high vacuum sintering furnace to obtain sintered magnet.

5. The preparation process of claim 4, further comprising that the molded preform is primarily tempered at 850-950 °C for 2-3 hours and/or secondarily tempered at 450-550 °C for 2-5 hours.

## Patentansprüche

1. Herstellungsverfahren für einen hoch korrosionsbeständigen NdFeB-Sintermagneten, wobei das Verfahren Folgendes umfasst:
Bereitstellen eines Hauptphasenlegierungspulvers, wobei die Zusammensetzung der Hauptphasenlegierung in Massen-% NdₓRₓ₁Fe_{100-(x+x1+y+z)}T_{y}B_{z} lautet, wobei 24 ≤ x ≤ 33, 0 ≤ x1 ≤ 15, 1,43 ≤ y ≤ 16,43, 0,91 ≤ z ≤ 1,07, R für ein oder mehrere Elemente aus der Gruppe bestehend aus Dy, Tb, Pr, Ce und Gd steht und T für ein oder mehrere Elemente aus der Gruppe bestehend aus Co, Cu und Al steht;
Bereitstellen eines Hilfsphasenlegierungspulvers;
Mischen des Hauptphasenlegierungspulvers mit dem Hilfsphasenlegierungspulver, wobei der Gehalt des Hilfsphasenlegierungspulvers 1-10 % der Gesamtmasse beträgt;
Formpressen des gemischten Pulvers in einem Magnetfeld zu einer Vorform und anschließendes isostatisches Pressen bei einem Druck über 200 MPa;
Einbringen der geformten Vorform in einen Hochvakuum-Sinterofen zum Sintern zum Erhalt eines Sintermagneten, wobei die Gruppe refraktärer Metalle hauptsächlich in der Korngrenzenphase des NdFeB-Magneten verteilt ist,
**dadurch gekennzeichnet, dass** die Zusammensetzung der Hilfsphasenlegierung in Massen-% NdₓRₓ₁Fe_{100-(x+x1+y+y1+z)}T_{y}M_{y1}B_{z} lautet, wobei 24 ≤ x ≤ 63, 0 ≤ x1 ≤ 19, 1,43 ≤ y ≤ 16,43, 6 ≤ y1 ≤ 18, 0,91 ≤ z ≤ 1,07, der Gehalt an Fe 100 - (x + x1 + y + y1 + z) beträgt, R für ein oder mehrere Elemente aus der Gruppe bestehend aus Dy, Tb, Pr, Ce und Gd steht, T für ein oder mehrere Elemente aus der Gruppe bestehend aus Co, Cu und Al steht und M für ein oder mehrere Metalle aus der Gruppe refraktärer Metalle, die aus Nb, Zr, Ti, Cr und Mo besteht, steht.

2. Herstellungsverfahren nach Anspruch 1, wobei der mittlere Teilchendurchmesser des Hauptphasenlegierungspulvers 2-5 µm beträgt.

3. Herstellungsverfahren nach Anspruch 1, wobei der mittlere Teilchendurchmesser des Hilfsphasenlegierungspulvers 2-5 µm beträgt.

4. Herstellverfahren nach Anspruch 1, wobei die geformte Vorform zum Erhalt eines Sintermagneten im Hochvakuum-Sinterofen 2-5 Stunden bei 1040-1120 °C gesintert wird.

5. Herstellungsverfahren nach Anspruch 4, ferner umfassend, dass die geformte Vorform 2-3 Stunden bei 850-950 °C primär getempert wird und/oder 2-5 Stunden bei 450-550 °C sekundär getempert wird.

## Revendications

1. Procédé de préparation d'un aimant de NdFeB fritté hautement résistant à la corrosion, ledit procédé comprenant :
la mise à disposition d'une poudre d'alliage de phase principale, la composition de l'alliage de phase principale en % en masse étant NdₓRₓ₁Fe_{100-(x + x1 + y + z)}T_{y}B_{z}, 24 ≤ x ≤ 33, 0 ≤ x1 ≤ 15, 1,43 ≤ y ≤ 16,43, 0,91 ≤ z ≤ 1,07, R étant l'un ou plusieurs choisis dans le groupe constitué par Dy, Tb, Pr, Ce et Gd, T étant l'un ou plusieurs choisis dans le groupe constitué par Co, Cu, et Al ;
la mise à disposition d'une poudre d'alliage de phase auxiliaire ;
le mélange de la poudre d'alliage de phase principale avec la poudre d'alliage de phase auxiliaire, la teneur en poudre d'alliage de phase auxiliaire étant de 1 à 10 % de la masse totale ;
le moulage par pressage de la poudre mélangée dans un champ magnétique en une préforme, ensuite une compression isostatique a été réalisée à une pression supérieure à 200 MPa ;
le placement de la préforme moulée dans un four de frittage sous vide poussé, afin d'obtenir un aimant fritté, le groupe de métaux réfractaires étant principalement distribué dans la phase intergranulaire de l'aimant NdFeB,
**caractérisé en ce que** la composition de l'alliage de phase auxiliaire en % en masse est NdₓRₓ₁Fe_{100-(x + x1 + y + y1 + z)}T_{y}M_{y1}B_{z}, 24 ≤ x ≤ 63, 0 ≤ x1 ≤ 19, 1, 43 ≤ y ≤ 16,43, 6 ≤ y1 ≤ 18, 0,91 ≤ z ≤ 1,07, la teneur en Fe étant de 100 - (x + x1 + y + y1 + z), et R étant l'un ou plusieurs choisis dans le groupe constitué par Dy, Tb, Pr, Ce et Gd, T étant l'un ou plusieurs choisis dans le groupe constitué par Co, Cu, et Al, M étant l'un ou plusieurs choisis dans le groupe de métaux réfractaires constitué par Nb, Zr, Ti, Cr et Mo.

2. Procédé de préparation selon la revendication 1, le diamètre moyen de particule de la poudre d'alliage de phase principale étant de 2 à 5 µm.

3. Procédé de préparation selon la revendication 1, le diamètre moyen de particule de la poudre d'alliage de phase auxiliaire étant de 2 à 5 µm.

4. Procédé de préparation selon la revendication 1, la préforme moulée étant frittée à une température de 1 040 à 1 120 °C pendant 2 à 5 heures dans un four de frittage sous vide poussé pour obtenir un aimant fritté.

5. Procédé de préparation selon la revendication 4, comprenant en outre le fait que la préforme moulée est principalement trempée à une température de 850 à 950 °C pendant 2 à 3 heures et/ou secondairement trempée à une température de 450 à 550 °C pendant 2 à 5 heures.
